

(No Model.)

C. GRAHAM.  
PROCESS OF MAKING CROCKERY WASH TUBS.

No. 436,413.

Patented Sept. 16, 1890.

Fig. 1.



Fig. 2.



Fig. 3.



Fig. 4.



Witnesses:

Charles R. Searle.  
H. J. Johnstone.

Inventor:

Charles Graham  
by his attorney  
Thomas D. Newell, Stetson

# UNITED STATES PATENT OFFICE.

CHARLES GRAHAM, OF BROOKLYN, NEW YORK.

## PROCESS OF MAKING CROCKERY WASH-TUBS.

SPECIFICATION forming part of Letters Patent No. 436,413, dated September 16, 1890.

Application filed July 20, 1888. Serial No. 280,463. (No model.)

*To all whom it may concern:*

Be it known that I, CHARLES GRAHAM, of Brooklyn, Kings county, in the State of New York, have invented a certain new and useful Improvement in Crockery Wash-Tubs, of which the following is a specification.

It has been found practicable to make rectangular vessels with inclined front sides suitable for stationary wash-tubs by shaping them, 10 with suitable precautions, in wet clay, drying and burning in kilns in the same manner as other crockery articles. I do the same. It is desirable that such tubs shall present a clear white interior surface. This has been heretofore attained by making them entirely of 15 clay which burns white. An objection to such lies in the great fragility before burning while in the condition known as "biscuit." It involves great care in the handling and 20 risk of much loss by breakage.

It has long been known that pottery articles may be made of clay which will burn yellow or brown, and lined with a wash of clay which burns white. Small articles, as pipkins, have 25 long been made in that manner, the biscuit being tough and able to endure rougher handling than all-white ware. An objection to such compound construction of the crockery lies in the liability of the thin coating to 30 flake off in the burning or at some subsequent period while the article is in use.

I have discovered means for insuring the adhesion of the thin coating of white clay to a body of cheaper and tougher biscuit. By 35 this means I am able to produce wash-tubs having their main bodies of clay, which is lower in cost and maintains its integrity more reliably in the handling which is necessary previous to the burning, and which, although 40 presenting unattractive tints, various shades and streaks of dull yellow, red, and brown on the exterior, are white and clear on their inner faces, the only surfaces where these qualities are important. I produce the bottom 45 and four sides of the tub from properly-made slabs of evenly-worked tough clay, and by thoroughly kneading the junctions effect a reliable union. I treat such body by pressure in dies or otherwise to bring it to the exact 50 size and form desired, a little larger than the finished tub required, to allow for shrinking. So far the manipulation is the same as

with ordinary crockery wash-tubs, except that I am indifferent with regard to the color of the main body, but only anxious to secure a tough 55 biscuit, the shrinkage of which in burning shall be, as nearly as possible, equal to that of the white ware with which its interior is to be lined. The body thus formed is exposed to the air in the shade until it is nearly, but not quite, 60 dry. Its condition may be described as leathery. Practice will be required to determine when this point is reached. It is important that the clay be sufficiently dry to have much strength, and yet that it be sufficiently damp 65 to have its inner surface rapidly softened on the reception of the wet coating to be applied there. Now, having worked with clear water to the consistency of cream a liberal quantity of white clay—by which I mean that 70 which will produce white crockery or analogous white ware when burned—I apply it rapidly and as uniformly as practicable in a thin coating, covering the entire interior. I have, in my experiments, effected this by 75 distributing the material roughly on the inner surfaces from a cup or other vessel, and then immediately spreading it by a brush. The nearly-dried biscuit will absorb the moisture from this coating, so that it will dry 80 rapidly, and in a short time—two or three hours, more or less—it will be so far dried as to be ready for a second coating. This is applied in the same manner. The water from this second coat will soften the first coat and 85 also the adjacent portion of the main body. When this softening has reached a certain stage, determined by practice—say about one or two hours, under the conditions which obtain in the dry atmosphere in this country in 90 clear weather—I treat the whole inner surface by rubbing first with a piece of vulcanized soft rubber held at an inclination and drawn over the entire surface several times, moving up and down and horizontally on all the four 95 sides and similarly cross wiping or rubbing the bottom. A strong pressure is applied on this rubber during the early stages of the treatment; but the pressure is gradually lessened as it proceeds, until it is finished with 100 very light wiping. A little later in the drying operation the whole surface is slicked with a large knife. The pressure applied during this treatment also should be firm at

the commencement and grow less as the work proceeds. The biscuit thus lined, with the lining compressed upon and into intimate union with the main body, is now allowed to dry further, and is subsequently glazed and burned, care being taken to keep the smoke of the kiln from the interior in the same manner as with all white ware. I believe that the rubbing has an effect analogous to the kneading by which potters have long joined separately-formed parts of crockery-ware, and by which the five separate flat slabs employed in building up the body of this kind of tubs are joined.

I am not aware that a lining has before been compressed upon a body by such treatment or by any analogous treatment. My experiments indicate that the lining produced by two coats of the creamy-white clay applied in this manner and compressed on the body with patient manipulation is sufficiently thick to produce substantially the same effect on the eye as clear white ware, and is reliably joined, so that it will endure all the ordinary and extraordinary treatment to which the tub is subjected in storage, transportation, and use.

The accompanying drawings form a part of this specification.

Figure 1 is a cross - section of the completed tub. The remaining figures are on a larger scale. Fig. 2 is a cross-section showing a portion of the tub before the lining is applied. Fig. 3 is a cross-section showing a portion of the tub after the lining is applied and before the rubbing. Fig. 4 is a corresponding section showing the condition attained after the rubbing has effected the required intimate union.

In all the figures, A is the main body, B the

white-ware lining, and c the junction. Before the rubbing the junction c is smooth and incomplete. After the rubbing it is irregular, the particles of the one being impressed into and partially interwoven with the particles of the other material. 40

Modifications may be made in the details without departing from the principle or sacrificing the advantages of the invention. I can smooth with the rubber the whole interior of the body before applying the first coat, 50 and again after applying the first coat before applying the second. My experiments indicate that there are some advantages in doing this; but I do not esteem such rubbings previous to the rubbing on the final coat essential to success. 55

I claim as my invention—

The method described of uniting a lining of white-burning clay with a body of tougher clay by first shaping and partly drying the body A of tough clay and preparing the white-burning clay in a semi-fluid or creamy condition, then applying the semi-fluid clay as a wash to the inside of the vessel in one or more coats, allowing it to stand a sufficient time to 60 allow the moisture to become nearly or quite equalized throughout the whole interior portion of the vessel, and then agitating the particles and blending them by rubbing, as herein specified. 65

In testimony whereof I have hereunto set my hand, at New York city, this 19th day of July, 1888, in the presence of two subscribing witnesses.

CHAS. GRAHAM.

Witnesses:

THOMAS DREW STETSON,  
H. A. JOHNSTONE.

70